

Nov. 11, 1958

N. H. BRUNDIN

2,860,044

METHOD IN THE PRODUCTION OF IRON POWDER OF DESIRED GRAIN SIZE

Filed Feb. 20, 1951



Inventor

Nils Herman Brundin  
Puice, Scheffler & Parker  
attys

## 1

2,860,044

**METHOD IN THE PRODUCTION OF IRON  
POWDER OF DESIRED GRAIN SIZE**

Nils H. Brundin, Hoganas, Sweden, assignor to Hoganas-Billesholms Aktiebolag, Hoganas, Sweden, a corporation of Sweden

Application February 20, 1951, Serial No. 211,982

3 Claims. (Cl. 75—5)

When sponge iron is produced from oxide in powder form, especially if coke or charcoal is used as reducing agent, the temperature must, in practice, be so high that the sponge iron is obtained as hard, sintered cakes of considerable strength. These cakes can, after crushing, be ground to a powder. Such sponge iron powder can be used for powder metallurgical purposes if certain conditions are fulfilled. These are:

- (1) The powder must pass a 100 mesh screen.
- (2) The volume weight must not exceed 2.5, which means that the milling must be done in such a way that the grains substantially retain their original porous structure.

Because of this latter reason the grinding must be done very carefully and in practice it has been shown that some conventional mills are not suitable for the purpose. Two types of mills which have been found suitable are the pan mill and the disintegrator in which the treatment is mild enough to let the grains retain their porous structure after milling.

In practice it was found, however, that it was not possible to grind sponge iron cakes in these mills so that all powder obtained was suitable for use for powder metallurgical purposes. About 20% of the obtained powder would not pass a 100 mesh screen and even if this 20% was recirculated it was not possible to reduce the size any further. Therefore this 20% had to be used for other purposes. It is possible to grind this powder to a finer grain size in a ball mill but even then the powder is not suitable for use in the powder metallurgy because by this treatment the volume weight becomes much higher than the allowed 2.5.

The purpose of this invention is to make possible a more complete conversion of the hard, sintered cakes to a powder suitable for use in powder metallurgy and thus to decrease the up to now unavoidable loss in said powder which will not pass a 100 mesh screen.

The invention is based on the discovery that the grain size of the iron oxide used as raw material for the sponge iron production has a considerable influence on the production of a powder of wanted grain size. This is rather astonishing since the reduction has to be carried out at a temperature considerably higher than the temperature at which a crystallization and grain growth of iron takes place, wherefore it was to be expected that the original grain boundaries would disappear and be without influence on the grindability. Further each original grain has a considerable porosity which ought to decrease the mechanical strength and make it possible to split it up in the grinding process.

According to the invention the iron oxide which is to be used for powder production is, by suitable means such as grinding or sieving, reduced to a grain size which is

## 2

the same as or less than the grain size desired in the iron powder, whereafter the oxide powder is reduced to sponge iron, which after cooling and crushing is milled to the wanted grain size.

- 5      *Example.*—Magnetite concentrate was mixed with powdered charcoal in the proportions 100:33 and the mixture heated to 1000° C. where it was kept until the reduction was complete. After cooling the obtained sponge iron was crushed in a jaw-crusher and milled in a disintegrator.
- 10     After milling the powder was screened on a 100 mesh sieve and the powder not passing the sieve was milled again. This treatment was repeated several times and the different fractions weighed.

One experiment was carried out with a magnetite concentrate passing 40 mesh and one with concentrate passing 100 mesh.

The result is given in the accompanying drawing where the accumulative percentage of powder passing 100 mesh is shown as a function of the number of milling operations.

As is seen from the drawing the unavoidable loss when using 40 mesh concentrate amounted to about 20 percent whereas the corresponding loss when using 100 mesh concentrate as starting material only amounted to about 2.5 percent.

We claim:

1. A method for the production of iron powder of the desired grain size for powder metallurgical purposes which comprises mechanically reducing an iron oxide ore to a particle size not greater than said desired grain size, chemically reducing said iron oxide ore to iron powder at a temperature sufficient to produce sponge iron in the form of hard, sintered cakes, cooling said cakes and comminuting them to a powder of said desired grain size.
- 30     2. A method for the production of iron powder as defined in claim 1 in which the iron oxide ore is of a grain size capable of passing a 100 mesh screen, is free of carbonizable liquid, is reduced in the presence of a solid reducing agent and at least about 97.5% of the powder produced by comminuting will pass a 100 mesh screen and has a volume weight not greater than about 2.5.
- 45     3. A method for the production of iron powder of about 100 mesh and suitable for powder metallurgy which comprises mechanically reducing iron ore of greater particle size to not greater than about 100 mesh, chemically reducing the resulting ore at a temperature sufficient to produce sponge iron in the form of a hard, sintered cake and cooling and disintegrating said sponge iron cake to about 100 mesh.

**References Cited in the file of this patent**
**UNITED STATES PATENTS**

|           |                        |               |
|-----------|------------------------|---------------|
| 2,200,491 | Cross et al. -----     | May 14, 1940  |
| 2,216,770 | Drapeau et al. -----   | Oct. 8, 1940  |
| 2,252,697 | Brassert -----         | Aug. 19, 1941 |
| 2,279,013 | Roseby -----           | Apr. 7, 1942  |
| 2,402,120 | Boegehold et al. ----- | June 18, 1946 |
| 2,413,492 | Firth -----            | Dec. 31, 1946 |

**FOREIGN PATENTS**

|         |                     |               |
|---------|---------------------|---------------|
| 568,786 | Great Britain ----- | Apr. 20, 1945 |
|---------|---------------------|---------------|

**OTHER REFERENCES**

65     Powder Metallurgy, page 119. Edited by Wulff. Published in 1942 by the American Society for Metals, Cleveland, Ohio.